

## UNITED STATES PATENT OFFICE.

HENRY PHILIP SHOPNECK, OF DORCHESTER, MASSACHUSETTS, ASSIGNOR TO JOHN J. DALY, OF WEST NEWTON, MASSACHUSETTS.

## FELTED BOX-TOE STOCK AND METHOD OF MAKING THE SAME.

No Drawing.

Application filed July 31, 1925. Serial No. 47,871.

REISSUED

*To all whom it may concern:*

Be it known that I, HENRY P. SHOPNECK, a citizen of the United States, residing at Dorchester, county of Suffolk, Commonwealth of Massachusetts, have invented certain new and useful Improvements in Felted Box-Toe Stocks and Methods of Making the Same, of which the following is a specification.

10 Various substitutes have been proposed for the expensive wool felt used in box toe stock in the effort to produce a low-cost, durable box toe material which will be sufficiently absorbent to take up and retain the thermo-plastic binder, which will possess sufficient tensile strength to hold its shape under the severe strains in lasting the shoe, and which will not only have capacity for stretch to assume the shape of the toe but will be 20 sufficiently resilient to return to shape after compression. Paper felt containing hair has been proposed, but so far as I am advised, nothing has been found as a substitute for animal hair to give the required 25 strength to such box toe stock. The cost of hair is, however, very high and makes factory material sometimes hard to obtain. Hair is furthermore difficult to work in the stock and run on a cylinder machine.

30 To the end, therefore, of producing a box toe stock which will embody the foregoing requisites while entirely avoiding the use of hair and wool felt, I have devised my present invention. According to it, I take 35 a fibrous pulp, such as waste textile rags (mixed rags containing more or less wool) or a mixture of such rags and wood pulp or other fibres, and beat it out until smooth. To this I add relatively long vegetable fibres, 40 such as jute, manila, hemp, or sisal, and then smooth out the mixture without cutting the long vegetable fibres.

I obtain the vegetable fibres from usual sources, and they are preferably loosely fiberized before incorporation into the mix.

45 The mix is beaten out in a paper maker's beater and run on a cylinder machine. I thus obtain a water-laid felt in which the long vegetable fibres are uniformly distributed throughout the body of short fibrous pulp and in felted relation therewith. Where the felt is used for box toes, the resultant dry sheet is then impregnated with 50 a thermoplastic binder, such as a mixture of hardened rosin and oil-blown asphalt, by

dipping the sheet of felt material into a fluid bath containing the thermo-plastic compound.

By using vegetable fibres, instead of animal hair, as has been proposed heretofore, I obtain a mix which not only felts better, but is stronger and can be more easily moulded on a last. It is common knowledge that animal hair of itself does not "felt," as this term is used in referring to the forming of stock into sheets by means of a cylinder machine, whereas jute has a felting action. A satisfactory felt is obtained by using a furnish consisting of approximately 30% jute or other relatively 70 long vegetable fibre and 70% rag or other fibrous stock.

If desired, I may increase the proportion of vegetable fibre to rags while retaining all the advantages of increased tensile 75 strength, by substituting for a portion of the rag stock, an equivalent portion of asbestos or other fibres, a characteristic mix consisting of approximately, 50% rag stock, 30% vegetable fibres, and 20% asbestos. It 80 is to be understood that what is meant by long vegetable fibres are the elongated fibres composed of a plurality of bundles of fibres which owe their adhesion to the encrusting effect of the ligneous constituents 85 on the intercellular substances. It is also to be understood that what is meant by the terms "fibrous pulp" and "body of short felted fibre," is a base of cotton, textile rags, news, wood pulp, or asbestos, or similar 90 fibres, with or without inert filler, or suitable mixtures of them.

These and various other modifications in materials and proportions, coming within the spirit and scope of my invention as defined by the appended claims, may obviously 95 be resorted to.

What I therefore claim and desire to secure by Letters Patent is:

1. A felt, consisting of a fibrous pulp, and relatively longer vegetable fibres and asbestos distributed throughout the mass in felted relation therewith and capable of being impregnated with a thermo-plastic binder. 100
2. A felt, consisting of a fibrous pulp, and relatively longer jute fibres and asbestos distributed throughout the mass in felted relation therewith and capable of being impregnated with a thermo-plastic binder. 105
3. A felt, consisting of a fibrous pulp and 110

- relatively longer jute fibres and asbestos distributed throughout the mass in felted relation therewith and capable of being impregnated with a thermo-plastic binder,
- 5 the proportion of vegetable fibres and asbestos each being substantially less than that of the fibrous pulp.
4. The method of making a felted stock, which consists in forming a sheet from a beaten fibrous pulp to which has been added relatively longer vegetable fibres of the class
- 10 described and asbestos, and in subsequently impregnating said sheet with a thermo-plastic binder.
5. A box toe material, comprising a fibrous pulp and relatively longer vegetable fibres and asbestos distributed throughout the mass in felted relation and impregnated with a thermo-plastic binder.

In testimony whereof I affix my signature.

HENRY PHILIP SHOPNECK.